

## UNITED STATES PATENT OFFICE

2,575,196

MIXED ESTERS OF POLYHYDRIC ALCOHOLS  
AND DIBASIC ACIDSPaul V. Smith, Jr., Westfield, N. J., assignor to  
Standard Oil Development Company, a corpora-  
tion of DelawareNo Drawing. Application October 1, 1948,  
Serial No. 52,430

7 Claims. (Cl. 260—485)

**1**  
This invention relates to a new class of compounds which have been particularly suitable for use as synthetic lubricants because of their low pour points and high viscosity indices.

In the lubricant art, considerable progress has been realized in recent years in the production of lubricants characterized by one or more specific properties and adapted for particular uses. In the main, this progress can be attributed to two developments: the first, new refining procedures, and the second, addition agents capable of imparting particular properties to available lubricants. Thus, viscosity index improvers and pour depressants are added to automotive lubricants to render the lubricants more adaptable to wide changes in temperature conditions, while other agents are added to improve the load-carrying properties of a lubricant which is to be employed, from example, under extreme pressure conditions.

Recently, in an effort to obtain superior lubricants endowed with specific and superior characteristics, a new field has been explored, namely the synthesis of lubricants from various materials. Esters represent one class of materials which have attracted unusual interests as synthetic lubricants. In general, they are characterized by higher viscosity indices and lower pour points than mineral oils of corresponding viscosity. The esters described in the present specification have been found to exhibit very low pour points, and high viscosity indices. Lubricants possessing such properties are of special value in the lubrication of engines which are subjected to high temperatures such as combustion turbine engines, particularly those of the "prop-jet" type. Mineral oil lubricants containing added viscosity index improvers, thickeners or other highly non-volatile additives are undesirable for use in such engines because of the tendency to leave a residue which accumulates and interferes with the operation of the engine. A synthetic lubricant of the type described in the present specification is especially adapted to use under such conditions, since the lubricant contains no additives and thus tends to leave no residue upon volatilization.

The new compounds of the present invention

**2**  
which have been found to be particularly suitable for use as lubricating oils are complex esters prepared by reacting one molecular proportion of a monobasic aliphatic acid with one molecular proportion of a glycol, thereby forming a half ester of the glycol, after which two molecular proportions of such half ester are reacted with one molecular proportion of a dibasic aliphatic acid. The esters are formed by simple reaction of the component parts, without heating or otherwise treating the product to form a polymerized or resinous material. It is usually desirable to employ an esterification catalyst such as p-toluenesulfonic acid. The reactions are conducted by the usual esterification methods, removing water as formed, as by means of a water trap attached to a refluxing condenser. A reaction medium or water-entraining medium, such as naphtha, benzene, toluene, or the like, is usually employed.

The new class of compounds may be broadly defined by the following general formula:



where  $\text{R}_1$  and  $\text{R}'_4$  are glycol radicals which may consist of saturated aliphatic hydrocarbon groups, straight chain or branched, containing 2 to 20 carbon atoms each, or they may each represent a series of saturated aliphatic hydrocarbon radicals interlinked by one or more oxygen or sulfur atoms, or both oxygen and sulfur atoms, provided there are at least two carbon atoms between each carboxyl group and the nearest oxygen or sulfur atom and at least two carbon atoms between each pair of oxygen and/or sulfur atoms in the chain, and provided further that the total number of carbon, oxygen and sulfur atoms in each radical is from 5 to 80 and the number of sulfur atoms in each radical is not greater than two.  $\text{R}_2$  and  $\text{R}'_3$  of the formula each represent

an aliphatic hydrocarbon radical, straight chain or branched, saturated or unsaturated, containing 1 to 22 carbon atoms, or they may represent organic radicals consisting of groups of short aliphatic hydrocarbon radicals interlinked by oxygen atoms, provided that the number of oxygen atoms in each radical is not greater than 5 and provided that there is at least one carbon atom between the carboxyl group and the first oxygen atom and at least two carbon atoms between each pair of oxygen atoms, the total number of carbon and oxygen atoms in the radical being from 3 to 22, or the radicals R<sub>2</sub> and R<sub>2'</sub> may represent organic radicals each consisting of an aliphatic hydrocarbon chain containing a single interlinking sulfur atom, such sulfur atom being separated from the carboxyl group by at least one carbon atom, the total number of carbon and sulfur atoms in the radical being from 3 to 22, R<sub>3</sub> of the formula is an aliphatic hydrocarbon radical, straight chain or branched, saturated or unsaturated, containing 0 to 30 carbon atoms, or it may be an organic radical consisting of a series of saturated aliphatic hydrocarbon radicals interlinked by one or more atoms of oxygen or sulfur, or both oxygen and sulfur, provided there are at least two carbon atoms between each pair of oxygen or sulfur atoms, provided there are not more than two sulfur atoms in each chain, provided there is at least one carbon atom between the carboxyl group and the first oxygen or sulfur atom, and provided that the total number of carbon, oxygen, and sulfur atoms in the entire radical R<sub>3</sub> is from 3 to 80. The molecular weight of the entire ester should be at least 300 and the viscosity at 210° F. should not be greater than 150 seconds (Saybolt) to provide a product having lubricating properties.

Among the various components of the complex esters of the present invention, certain preferences may be pointed out as giving the optimum of desired properties from the standpoint of service as a lubricant. The preferred glycols are the polyethylene glycols of the formula



where n is 1 to 26. The preferred monobasic acids are the fatty acids containing 2 to 10 carbon atoms per molecule. The preferred dibasic acids are the straight chain dibasic acids of the paraffinic group having from 6 to 10 carbon atoms per molecule.

Among the monobasic acids which may be employed in the preparation of the esters of the present invention the following may be listed as illustrative:

Acetic acid  
Propionic acid  
Butyric acid  
Valeric acid  
Caproic acid  
Caprylic acid  
Lauric acid  
Palmitic acid  
Stearic acid  
Oleic acid  
 $\beta$ -Methoxypropionic acid  
 $\beta$ -Ethoxypropionic acid  
 $\beta$ -tert.-Octoxypropionic acid  
 $\beta$ -Ethylmercaptopropionic acid  
 $\beta$ -tert.-Octylmercaptopropionic acid  
 $\beta$ -tert.-Dodecylmercaptopropionic acid

The glycols employed in preparing the esters of the present invention include ethylene glycol and any of the paraffinic homologues of the same

containing up to 20 carbon atoms. These may include, for example, ethylene glycol, propylene glycol, butylene glycols, pinacone, trimethylene glycol, tetramethylene glycol, pentamethylene glycol, and the like. Since the glycols may also contain oxygen or sulfur atoms, compounds such as diethylene glycol, triethylene glycol, the polyethylene glycols of the formula



where n is 1 to 26, and the polypropylene glycols of the general formula



where R<sub>1</sub> or R<sub>2</sub> is a methyl group and the other is hydrogen, and where n is 1 to 20, may likewise be employed. Glycols containing sulfur atoms in thioether linkages may also be employed, and these include such compounds as thiodiglycol and 1,2-bis(2-hydroxyethylmercapto)ethane. There also may be used glycols containing both oxygen and sulfur in similar linkages; such a compound is bis-[2-(2-hydroxyethoxy)ethyl]sulfide.

Illustrative examples of the dibasic acids which may be employed in the synthesis of the complex esters of the present invention are the following:

Oxalic acid

Malonic acid

Succinic acid

Glutaric acid

Adipic acid

Pimelic acid

Suberic acid

Azelaic acid

Sebatic acid

Brassylic acid

Pentadecanedicarboxylic acid

Tetracosanedicarboxylic acid

C<sub>4</sub>—C<sub>24</sub> Alkenylsuccinic acids

Diglycolic acid

Thiodiglycolic acid

The C<sub>4</sub>—C<sub>24</sub> alkenyl succinic acids listed above are prepared by condensing olefins or mixtures of olefins with maleic anhydride.

If desired, various addition agents may be incorporated in the esters of the present invention for the purpose of improving their properties with respect to their usefulness as lubricants. For example, antioxidants, viscosity index improvers, thickeners, dyes, etc., may be added.

Data will be given below showing the preparation of several examples of complex esters within the scope of the present invention, indicating the adaptability of these esters to lubricating service. All of these esters were prepared by a general esterification method which may be described in detail as follows: In a 1-liter round bottom reaction flask, fitted with a reflux condenser and water trap, were placed one mol of monobasic acid, one mol of glycol, 2.5 grams of p-toluenesulfonic acid monohydrate (catalyst), and 100 ml. toluene. The mixture was refluxed until no more water collected in the water trap. After cooling, 0.5 mol of dibasic acid was added and the refluxing process resumed until again no more water collected in the trap. The mixture was washed with three 100 ml. portions of saturated aqueous sodium carbonate solution and one 100 ml. portion of water. After drying with "Drierite" (anhydrous calcium sulfate) the material was filtered and stripped at a pressure of about 5 mm. to a bath temperature of about 225° C.

The results of tests of various properties of

esters prepared by the above general method are shown in the table of data as follows:

2. A composition according to claim 1 in which  $R_1$  and  $R_1'$  represent radicals of the formula

| Component of Ester                | Flash Point<br>(° F.) | Kinematic Viscosity |         | ASTM Slope | Viscosity Index | ASTM Pour Point<br>(° F.) |
|-----------------------------------|-----------------------|---------------------|---------|------------|-----------------|---------------------------|
|                                   |                       | 100° F.             | 210° F. |            |                 |                           |
| Valeric acid                      |                       |                     |         |            |                 |                           |
| Adipic acid                       | 435                   | 42.480              | 8.487   | 0.588      | 153             | <-35                      |
| Tetraethylene glycol              |                       |                     |         |            |                 |                           |
| Valeric acid                      |                       |                     |         |            |                 |                           |
| Adipic acid                       | 395                   | 30.030              | 6.346   | 0.628      | 157             | <-35                      |
| Triethylene glycol                |                       |                     |         |            |                 |                           |
| Caproic acid                      |                       |                     |         |            |                 |                           |
| Adipic acid                       | 460                   | 44.538              | 8.848   | 0.582      | 153             | <-35                      |
| Tetraethylene glycol              |                       |                     |         |            |                 |                           |
| Caprylic acid                     |                       |                     |         |            |                 |                           |
| Adipic acid                       | 475                   | 43.335              | 8.678   | 0.583      | 153             | <-35                      |
| Tetraethylene glycol              |                       |                     |         |            |                 |                           |
| Caprylic acid                     |                       |                     |         |            |                 |                           |
| Adipic acid                       | 470                   | 37.240              | 7.493   | 0.610      | 152             | <-35                      |
| Triethylene glycol                |                       |                     |         |            |                 |                           |
| Acetic acid                       |                       |                     |         |            |                 |                           |
| Sebatic acid                      |                       |                     |         |            |                 |                           |
| Tetraethylene glycol              | 440                   | 82.200              | 13.409  | 0.567      | 141             | <-35                      |
| Propionic acid                    |                       |                     |         |            |                 |                           |
| Sebatic acid                      |                       |                     |         |            |                 |                           |
| Tetraethylene glycol              | 415                   | 51.846              | 9.922   | 0.573      | 150             | <-35                      |
| Butyric acid                      |                       |                     |         |            |                 |                           |
| Sebatic acid                      |                       |                     |         |            |                 |                           |
| Tetraethylene glycol              | 435                   | 54.56               | 10.60   | 0.559      | 152             | <-35                      |
| Valeric acid                      |                       |                     |         |            |                 |                           |
| Sebatic acid                      |                       |                     |         |            |                 |                           |
| Tetraethylene glycol              | 445                   | 58.852              | 11.576  | 0.542      | 152             | <-35                      |
| Caproic acid                      |                       |                     |         |            |                 |                           |
| Sebatic acid                      |                       |                     |         |            |                 |                           |
| Tetraethylene glycol              | 465                   | 56.150              | 10.995  | 0.551      | 152             | <-35                      |
| Butyric acid                      |                       |                     |         |            |                 |                           |
| Thiodipropionic acid              |                       |                     |         |            |                 |                           |
| Thiodiglycol                      |                       |                     |         |            |                 |                           |
| Butyric acid                      |                       |                     |         |            |                 |                           |
| Thiodipropionic acid              | 375                   | 37.330              | 7.111   | 0.636      | 150             | <-35                      |
| Tetraethylene glycol              |                       |                     |         |            |                 |                           |
| Butyric acid                      |                       |                     |         |            |                 |                           |
| Thiodipropionic acid              | 390                   | 42.470              | 7.734   | 0.633      | 144             | -40                       |
| Tetraethylene glycol              |                       |                     |         |            |                 |                           |
| Butyric acid                      |                       |                     |         |            |                 |                           |
| Adipic acid (0.25 mol)            |                       |                     |         |            |                 |                           |
| Sebatic acid (0.25 mol)           |                       |                     |         |            |                 |                           |
| Tetraethylene glycol              |                       |                     |         |            |                 |                           |
| Acetic acid                       |                       |                     |         |            |                 |                           |
| Adipic acid                       |                       |                     |         |            |                 |                           |
| Ethylene glycol                   | 395                   | 116.3               | 14.030  | 0.631      | 121             | -15                       |
| Butyric acid                      |                       |                     |         |            |                 |                           |
| Adipic acid                       |                       |                     |         |            |                 |                           |
| Polyethylene glycol (300 mol wt.) | 435                   | 62.155              | 11.476  | 0.560      | 148             | -35                       |

The above data indicate that the esters constituting the subject matter of the present invention possess characteristics, particularly with regard to viscosity index and pour point, which indicate their suitability for general use as lubricating oils and particularly for use where the presence of additives is not desirable. The esters of the present invention may be blended with mineral lubricating oils to give lubricants of improved viscosity index and pour point.

What is claimed is:

1. As a new composition of matter a compound of the formula



where  $R_1$  and  $R_1'$  are radicals of the formula  $-(\text{CH}_2\text{CH}_2\text{X})_n\text{CH}_2\text{CH}_2$ — in which  $\text{X}$  is a member of the group consisting of oxygen and sulfur and  $n$  is an integer from 1 to 7; where  $R_2$  and  $R_2'$  are alkyl groups containing 1 to 7 carbon atoms each; and where  $R_3$  is a radical selected from a group consisting of (1) radicals of the formula  $-(\text{CH}_2)_m$ — where  $m$  is an integer from 4 to 8, (2) radicals of the formula  $-(\text{CH}_2)_n\text{O}(\text{CH}_2)_n$ — where  $n$  is an integer from 2 to 4, and (3) radicals of the formula  $-(\text{CH}_2)_p\text{S}(\text{CH}_2)_p$ — where  $p$  is an integer from 2 to 4.

— $(\text{CH}_2\text{CH}_2\text{O})_n\text{CH}_2\text{CH}_2$ — where  $n$  is an integer from 2 to 3.

45 3. A composition according to claim 1 in which  $R_3$  is a radical of the formula  $-(\text{CH}_2)_m$ — where  $m$  is an integer from 4 to 8.

4. A composition according to claim 3 in which  $m$  is 4.

50 5. As a new composition of matter a compound according to claim 1 in which  $R_1$  and  $R_1'$  of the formula each represent the radical



55  $R_2$  and  $R_2'$  of the formula each represent the radical



and  $R_3$  of the formula represents



60 6. A composition according to claim 1 in which  $R_1$  and  $R_1'$  of the formula represent radicals of the formula



65 in which  $R_2$  and  $R_2'$  of the formula represent methyl radicals, and in which  $R_3$  of the formula represents the radical



70 7. A composition according to claim 1 in which  $R_1$  and  $R_1'$  of the formula represent the radical



in which  $R_2$  and  $R_2'$  of the formula represent



and in which R<sub>3</sub> of the formula represents the radical

—(CH<sub>2</sub>)<sub>6</sub>—

PAUL V. SMITH, JR.

**REFERENCES CITED**

The following references are of record in the file of this patent:

**UNITED STATES PATENTS**

|   | Number    | Name          | Date          |
|---|-----------|---------------|---------------|
|   | 2,023,976 | Roberts       | Dec. 10, 1935 |
| 5 | 2,234,722 | Dickey et al. | Mar. 11, 1941 |
|   | 2,384,119 | Muskat        | Sept. 4, 1945 |